

# UNITED STATES PATENT OFFICE.

LEWIS S. EASTLAKE, OF CHICAGO, ILLINOIS.

## METHOD OF MAKING LUBRICATING-OILS.

1,352,502.

Specification of Letters Patent. Patented Sept. 14, 1920.

No Drawing.

Application filed December 7, 1917. Serial No. 205,948.

To all whom it may concern:

Be it known that I, LEWIS S. EASTLAKE, a citizen of the United States, and a resident of the city of Chicago, county of Cook, and 5 State of Illinois, have invented certain new and useful Improvements in Methods of Making Lubricating-Oils, of which the following is a specification.

My invention relates to improvements in 10 methods of making lubricating oils, and has for its object the provision of an improved method for this purpose whereby the waste or residue of ordinary lubricating oils may be utilized for making new oils.

15 The invention consists in the method hereinafter set forth and claimed.

The preferred method of procedure consists in collecting the ordinary waste residue of lubricating oil, such as is left in the 20 crank case of an ordinary gasoline engine, and which is usually thrown away. This spent residue consists substantially of the solvent portion of the oil from which practically all the lubricating portion has been 25 exhausted. The solid matter, such as the carbon and other impurities is removed from this residue preferably by filtration, as through a combined felt and paper filter, although this solid matter might perhaps be 30 removed by precipitation or by the use of centrifugal force. Then a suitable amount of lubricating element such as ordinary petrolatum or vaseline is mixed with this clarified residue, thus providing fresh lubricating 35 oil, which to all intents and purposes is as good as the original oil for lubricating purposes. To effect this mixture, the petrolatum or vaseline is preferably heated until it becomes quite liquid and then is mixed with

40 the clarified residue by stirring. To obtain a medium heavy oil I add about one pound of the petrolatum to one gallon of the clarified residue. If the proportion of petrolatum is increased a heavier oil may be produced, or if decreased a lighter oil produced, 45 so that the character of the lubricating oil produced may be varied as desired.

The lubricating oils thus produced are to all intents and purposes as good for lubricating purposes as was the original oil from 50 which the residue is obtained. Inasmuch as

this residue is ordinarily thrown away as of no further use, and the petrolatum or vaseline costs but little, lubricating oils may be produced by this process with great economy. 55

While I have set forth the preferred methods of procedure for carrying the invention into effect, these are capable of variation and modification without departing from the spirit of the invention. I, therefore, do not wish to be limited to the precise steps and proportion of parts set forth, but desire to avail myself of such variations and modifications as come within the scope of the appended claims. 60 65

Having described my invention what I claim as new and desire to secure by Letters Patent is:

1. The method of making lubricating oils which consists in mixing a lubricating element substantially free of solvents with the spent residue of used lubricating oil, substantially as described. 70

2. The method of making lubricating oils which consists in mixing petrolatum with the spent residue of used lubricating oil, substantially as described. 75

3. The method of making lubricating oils which consists in saving the spent residue of used lubricating oil; removing solid matter therefrom; and then mixing a lubricating element substantially free of solvents therewith, substantially as described. 80

4. The method of making lubricating oils which consists in saving the spent residue of used lubricating oil; removing solid matter therefrom; and then mixing petrolatum therewith, substantially as described. 85

5. The method of making lubricating oils which consists in filtering the spent residue of used lubricating oil; and then mixing a lubricating element substantially free of solvents therewith, substantially as described. 90

6. The method of making lubricating oils which consists in filtering the spent residue of used lubricating oil; and then heating and mixing a lubricating element substantially free of solvents therewith, substantially as described. 95

7. The method of making lubricating oils which consists in filtering the spent residue of used lubricating oil; and then mixing pet- 100

rolatum therewith, substantially as described.

8. The method of making lubricating oils which consists in filtering the spent residue of used lubricating oil; and then heating and mixing petrolatum therewith, substantially as described.

In testimony whereof I have signed my name to this specification in the presence of two subscribing witnesses.

LEWIS S. EASTLAKE.

Witnesses:

JOSHUA R. H. POTTS,  
B. G. RICHARDS.